

## United States Patent Office

2,955,087

Patented Oct. 4, 1960

1

2,955,087

COMPOSITIONS AND METHODS FOR TREATING  
METAL SURFACES

Charles H. Elbreder, 14 Lynnbrook Drive, Frontenac, Mo., assignor of one-fourth to Arthur D. Berryman, one-fourth to W. Gail Garner, and one-fourth to Edward J. Ross, all of Lemay, Mo.

No Drawing. Filed Apr. 8, 1957, Ser. No. 651,131

10 Claims. (Cl. 252—136)

This invention relates to compositions and methods for treating metal surfaces and more particularly to compositions and methods which are useful in the cleaning and removal of deposits from metal surfaces without adverse effect upon the metal, and to inhibited acid compositions and methods of inhibiting corrosion of a metal surface against the action of certain acids.

This application is a continuation-in-part of our pending application Serial No. 582,937, filed May 7, 1956, now abandoned.

Briefly, the invention is directed to a composition for treating a metal surface comprising hydrochloric acid, sulfuric acid, sulfamic acid or phosphoric acid and a compound selected from the group of compounds of the general formula:



wherein R represents a higher alkyl radical and X represents a halogen atom. The invention also includes inhibited acid compositions and novel methods of treating metal surfaces and inhibiting corrosion of metal surfaces.

Among the several objects of the invention may be noted the provision of compositions for treating metal surfaces; the provision of compositions of the class described which are useful to clean and remove deposits from metal surfaces without deleteriously affecting the metal or metal alloys present; the provision of compositions of this type in which the corrosive action of hydrochloric acid, sulfuric acid, sulfamic acid and phosphoric acid on metal and metal alloys is inhibited; the provision of novel inhibited acid compositions; the provision of convenient and economical methods for cleaning metal surfaces; and the provision of methods of inhibiting corrosion of a metal surface against the action of certain acids. Other objects and features will be in part apparent and in part pointed out hereinafter.

The invention accordingly comprises the products and methods hereinafter described, the scope of the invention being indicated in the following claims.

It has been common to employ acids such as hydrochloric acid, sulfuric acid, sulfamic acid and phosphoric acid in cleaning, pickling or removing oxides, scale and other acid-soluble deposits from metallic surfaces. While such acids are effective in removing deposits from the interior of water pipes, fittings and metallic surfaces generally, their use is objectionable since the acids frequently attack and corrode free metal surfaces exposed by the removal of the deposits. Various inhibitors have been developed to control the action of these acids against iron and other metals. However, none of the inhibitors used heretofore have been completely satisfactory in controlling the attack of these acids on metals, including zinc, zinc alloys, steel, copper and other metals. It is highly desirable to provide a composition for removing scale and

2

other deposits from these metal surfaces without adverse effect upon the metal or metal alloys. Also, it is very desirable to provide acid compositions which have inhibited corrosion activity and which, therefore, may be shipped and stored in conventional metal containers.

In accordance with the present invention, it has now been found that metal surfaces may be effectively cleaned and acid-soluble deposits removed therefrom without resultant attack or corrosion of the metal by means of a composition comprising hydrochloric acid, sulfuric acid, sulfamic acid or phosphoric acid and an isoquinolinium compound of the general formula:



15

wherein R represents a higher alkyl radical and X represents a halogen atom. It has also been found that the inclusion of one of these isoquinolinium compounds in the aforementioned acids gives inhibited compositions which may be shipped or stored in metal containers. The inclusion of small amounts of one of the isoquinolinium compounds of the class described above in the novel compositions of the invention effectively inhibits the corrosive action of the acid compound upon metals, but does not impair the action of the acid upon scale and other deposits commonly found upon metallic surfaces.

20 It is preferred that the isoquinolinium compound employed be one of the above formula wherein R is a higher alkyl radical having from 8 to 18 carbon atoms. Mixtures of such isoquinolinium compounds are also suitable for use in the practice of the invention. These isoquinolinium compounds are effective to inhibit the corrosive action of the commonly used acids, namely, hydrochloric acid, sulfuric acid, sulfamic acid and phosphoric acid.

25 Only a small amount of the isoquinolinium compounds described above is necessary to protect metal and metal alloys from attack by the acids employed for the removal of scale and acid-soluble deposits or to protect metal surfaces from corrosion during the shipment and storage of such acids. It is preferred that between approximately 0.01% to 2% by weight of the isoquinolinium compound, 30 based upon the weight of the acid compound, be included in the compositions of the invention. The amount of isoquinolinium compound employed may vary according to the particular acid used. Thus, amounts as small as 0.01% by weight of the isoquinolinium compound are sufficient to inhibit the action of sulfamic acid, whereas higher amounts, such as 1% by weight, for example, should be employed with compositions including sulfuric acid, hydrochloric acid or phosphoric acid.

35 The novel compositions of the invention are introduced into systems having metal surfaces, and are effective in removing acid-soluble deposits from such surfaces without corroding or otherwise affecting the metal in the surface. Also, the compositions may be used for other purposes for which the acid component is useful, the isoquinolinium compound therein serving to prevent corrosion of metal surfaces exposed to the acid component as during transportation and storage thereof. Moreover, it has been found that the usefulness of the compositions of the invention is not materially affected by heat or variations 40 in the concentration of the acid employed for removing scale deposits.

45 The following examples illustrate the invention.

## Example 1

50 A composition for treating a metal surface was prepared containing hydrochloric acid (6% by weight) and

lauryl isoquinolinium bromide (1% by weight, based upon the weight of the hydrochloric acid).

*Example 2*

A composition for treating a metal surface was prepared containing hydrochloric acid (6.5% by weight) and lauryl isoquinolinium bromide (0.2% by weight, based upon the weight of the hydrochloric acid).

*Example 3*

A composition for treating a metal surface was prepared containing sulfamic acid (6.5% by weight) and a mixture (0.5% by weight, based upon the weight of the sulfamic acid) of a major amount of lauryl isoquinolinium bromide and a minor amount of mixed alkyl isoquinolinium bromide compounds in which the alkyl groups contained from 8 to 18 carbon atoms.

*Example 4*

A composition for treating a metal surface was prepared containing sulfamic acid (6.5% by weight) and lauryl isoquinolinium bromide (0.01% by weight, based upon the weight of the sulfamic acid).

*Example 5*

A composition for treating a metal surface was prepared containing hydrochloric acid (6.5% by weight) and lauryl isoquinolinium chloride (1% by weight, based upon the weight of the hydrochloric acid).

*Example 6*

A composition for treating a metal surface was prepared containing hydrochloric acid (14% by weight) and lauryl isoquinolinium bromide (1% by weight, based upon the weight of the hydrochloric acid).

*Example 7*

An inhibited acid composition was prepared containing phosphoric acid (75% by weight) and lauryl isoquinolinium bromide (1% by weight, based upon the weight of the phosphoric acid).

*Example 8*

Two beakers, one containing the composition described in Example 1 (200 ml.) and the other containing hydrochloric acid (200 ml., 6% by weight) were employed, the latter beaker serving as a control. A galvanized steel strip test specimen (1" x 4") was placed in each beaker, and the time required for the galvanized coating to be stripped from the specimen was noted. In the case of the control beaker, the galvanized coating was completely stripped from the test specimen within ten minutes, whereas after a period of twenty-four hours there was no significant effect on the galvanized coating of the specimen in the beaker containing the composition of Example 1.

*Example 9*

Example 8 was repeated, except that one beaker contained the composition described in Example 3, and the control beaker contained sulfamic acid (6.5% by weight). It was found that the galvanized coating was completely stripped from the test specimen in the control beaker within forty-five minutes, whereas after a period of twenty-four hours there was no significant effect on the galvanized coating of the specimen in the beaker containing the composition of Example 3.

*Example 10*

Two beakers, one containing the composition described in Example 6 (800 ml.) and the other containing hydrochloric acid (800 ml., 14% by weight), were employed, the latter beaker serving as a control. A carbon steel strip test specimen (22 gauge 1" x 5") was placed in each beaker, and the weight loss determined after a period of 288 hours. It was found that the control

specimen lost 6.2078 grams, whereas the specimen in the beaker containing the composition of Example 6 lost only 0.0021 grams.

*Example 11*

5 Two beakers, one containing the composition described in Example 7 (800 ml.) and the other containing phosphoric acid (800 ml., 75% by weight), were employed, the latter beaker serving as a control. A carbon steel strip specimen (22 gauge 1" x 5") was placed in each beaker, and the weight loss of each strip was determined after a period of 288 hours. It was found that the control specimen lost 7.5454 grams, whereas the specimen in the beaker containing the composition of Example 7 lost only 0.0032 grams.

*Example 12*

Two beakers, one containing the composition described in Example 6 (800 ml.) and the other containing hydrochloric acid (800 ml., 14% by weight), were employed, the latter beaker serving as a control. A copper test specimen (1/8" x 1" x 5") was placed in each beaker, and the weight loss of the specimen was determined after a period of 72 hours. It was found that the control specimen lost 914 mg., whereas the specimen in the beaker containing the composition of Example 6 lost only 132 mg.

*Example 13*

Two beakers, one containing the composition described in Example 1 (800 ml.) and the other containing hydrochloric acid (800 ml., 6% by weight), were employed, the latter beaker serving as a control. A copper test specimen (1/8" x 1" x 5") was placed in each beaker, and the weight loss for each of the specimens was determined after a period of 72 hours. It was found that the control specimen lost 1724 mg., whereas the specimen in the beaker containing the composition of Example 1 lost only 95 mg.

*Example 14*

Static immersion tests were carried out by immersing 40 test strips of SAE 1010 steel in 77% solutions of phosphoric acid at 120° F. containing varying amounts of lauryl isoquinolinium bromide. It was found, on the basis of exposure for a 24-hour period, that the inclusion of 0.03% by weight of lauryl isoquinolinium bromide was sufficient to reduce the corrosion rate of the steel test strips to approximately 2.78 mils/year, whereas the corrosion rate of control strips of SAE 1010 steel in 77% phosphoric acid not containing lauryl isoquinolinium bromide amounted to over 1000 mils/year.

50 It will be understood that compositions containing hydrochloric acid, sulfuric acid, sulfamic acid or phosphoric acid and alkyl isoquinolinium halide compounds other than those mentioned above give results comparable to those described in the foregoing examples.

55 In view of the above, it will be seen that the several objects of the invention are achieved and other advantageous results attained.

As various changes could be made in the above methods and products without departing from the scope of 60 the invention, it is intended that all matter contained in the above description shall be interpreted as illustrative and not in a limiting sense.

I claim:

65 1. An acid composition having an inhibited corrosion activity relative to metal surfaces comprising an acid selected from the group consisting of hydrochloric acid, sulfuric acid, sulfamic acid and phosphoric acid, and approximately 0.01% to 2% by weight, based upon the weight of said acid compound, of a compound selected 70 from the group of compounds of the general formula:



wherein R represents an alkyl radical having from 8 to 18 carbon atoms and X represents a halogen atom.

2. An acid composition having an inhibited corrosion activity relative to metal surfaces comprising hydrochloric acid and approximately 0.01% to 2% by weight, based upon the weight of said acid, of lauryl isoquinolinium bromide.

3. An acid composition having an inhibited corrosion activity relative to metal surfaces comprising sulfuric acid and approximately 0.01% to 2% by weight, based upon the weight of said acid, of lauryl isoquinolinium bromide.

4. An acid composition having an inhibited corrosion activity relative to metal surfaces comprising sulfamic acid and approximately 0.01% to 2% by weight, based upon the weight of said acid, of lauryl isoquinolinium bromide.

5. An acid composition having an inhibited corrosion activity relative to metal surfaces comprising phosphoric acid and approximately 0.01% to 2% by weight, based upon the weight of said acid, of lauryl isoquinolinium bromide.

6. The method which comprises contacting a metal surface with a composition containing an acid selected from the group consisting of hydrochloric acid, sulfuric acid, sulfamic acid and phosphoric acid, and approximately 0.01% to 2% by weight, based upon the weight of said acid, of a compound selected from the group of compounds of the general formula:



wherein R represents an alkyl radical having from 8

to 18 carbon atoms and X represents a halogen atom.

7. The method which comprises contacting a metal surface with a composition containing hydrochloric acid and approximately 0.01% to 2% by weight, based upon the weight of said acid, of lauryl isoquinolinium bromide.

8. The method which comprises contacting a metal surface with a composition containing sulfuric acid and approximately 0.01% to 2% by weight, based upon the weight of said acid, of lauryl isoquinolinium bromide.

9. The method which comprises contacting a metal surface with a composition containing sulfamic acid and approximately 0.01% to 2% by weight, based upon the weight of said acid, of lauryl isoquinolinium bromide.

10. The method which comprises contacting a metal surface with a composition containing phosphoric acid and approximately 0.01% to 2% by weight, based upon the weight of said acid, of lauryl isoquinolinium bromide.

15

16. The method which comprises contacting a metal surface with a composition containing phosphoric acid and approximately 0.01% to 2% by weight, based upon the weight of said acid, of lauryl isoquinolinium bromide.

#### References Cited in the file of this patent

#### UNITED STATES PATENTS

|           |                 |               |
|-----------|-----------------|---------------|
| 1,678,775 | Gravell         | July 31, 1928 |
| 2,220,451 | Hunt            | Nov. 5, 1940  |
| 2,450,861 | Robinson        | Oct. 5, 1948  |
| 2,472,400 | Bond et al.     | June 7, 1949  |
| 2,606,873 | Cardwell et al. | Aug. 12, 1952 |
| 2,662,857 | Carroll         | Dec. 15, 1953 |
| 2,780,653 | Macy            | Feb. 5, 1957  |
| 2,814,593 | Beiswanger      | Nov. 26, 1957 |

#### FOREIGN PATENTS

|         |               |               |
|---------|---------------|---------------|
| 397,553 | Great Britain | Aug. 28, 1933 |
| 418,919 | Great Britain | Nov. 2, 1934  |

#### OTHER REFERENCES

Mann et al.: Ind. Eng. Chem., February 1936, p. 160.